

# United States Patent [19]

Koenig et al.

[11] 3,927,969

[45] Dec. 23, 1975

[54] INSECTPROOFING WOOL WITH ZINC ACETATE

[75] Inventors: **Nathan H. Koenig, Albany; Mendel Friedman, Moraga, both of Calif.**

[73] Assignee: **The United States of America as represented by the Secretary of Agriculture, Washington, D.C.**

[22] Filed: **Sept. 24, 1973**

[21] Appl. No.: **399,873**

[52] U.S. Cl..... **8/128 R; 8/127.6**

[51] Int. Cl.<sup>2</sup> ..... **D06M 3/02; D06M 13/00**

[58] Field of Search..... **8/128 R; 117/138.5; 424/289**

[56] **References Cited**

UNITED STATES PATENTS

1,921,926 8/1933 Jones ..... 424/289

|           |        |                   |         |
|-----------|--------|-------------------|---------|
| 2,400,377 | 5/1946 | Spearman .....    | 8/128   |
| 3,055,727 | 9/1962 | Koenig .....      | 8/128   |
| 3,079,215 | 2/1963 | Koenig .....      | 8/128   |
| 3,332,735 | 7/1967 | Koenig .....      | 8/128   |
| 3,867,095 | 2/1975 | Koenig et al..... | 8/128 R |

*Primary Examiner—Theodore Morris  
Attorney, Agent, or Firm—M. Howard Silverstein; W. Takacs*

[57] **ABSTRACT**

Wool is reacted with zinc acetate in the presence of a polar, high-boiling solvent, yielding a modified wool which has increased resistance to insects.

**4 Claims, No Drawings**

**INSECTPROOFING WOOL WITH ZINC ACETATE**

A non-exclusive, irrevocable, royalty-free license in the invention herein described, throughout the world for all purposes of the United States Government, with the power to grant sublicenses for such purposes, is hereby granted to the Government of the United States of America.

**DESCRIPTION OF THE INVENTION**

This invention relates to and has among its objects the provision of novel processes for modifying wool in order to increase its resistance to insects. Further objects of the invention will be evident from the following description wherein parts and percentages are by weight unless otherwise specified.

Although wool is a very useful fiber, it is subject to attack and destruction by insects, particularly moths and carpet beetles. Various treatments are available to protect wool from insect attack. Unfortunately, the known treatments suffer from such disadvantages as being cumbersome, time-consuming, non-durable, toxic, costly, or combinations of these.

The invention described herein provides a means for obviating the problems outlined above. In accordance with the invention, wool is reacted with zinc acetate in the presence of a special solvent, whereby there is formed a modified wool which exhibits increased resistance to insect attack.

A primary advantage of the invention is that it yields modified wool which is more resistant to insect attack than normal wool. Moreover, insect resistance is attained rapidly by a simple process. A further advantage of the invention is that the treatment is inexpensive.

Another advantage of the invention is that the improvement is essentially permanent. The treated wool does not lose its insect resistance after long use or repeated dry cleaning, but retains these properties for the life of the material.

A further advantage of the invention is that the modified wool retains its intrinsic properties so that it is useful for all the conventional applications as in fabricating garments, blankets, rugs, etc.

**DETAILED DESCRIPTION OF THE INVENTION**

In the process of the invention, wool is reacted with zinc acetate in the presence of a special polar, high-boiling solvent, namely, N,N-dimethylformamide (hereinafter referred to as DMF), N-methyl-2-pyrrolidinone, dimethyl sulfoxide, or ethylene glycol. The amount of solvent may be varied from about 1 to 20 parts thereof per part of wool. Generally, 4-8 parts of solvent per part of wool is sufficient and provides good results.

The amount of zinc acetate used in the reaction may be varied, depending on the degree of modification desired. Usually one uses about 0.2 to 3 parts thereof per part of wool.

The reaction is carried out at a temperature from 25° to 135°C. The rate of reaction increases with temperature, and it is preferred to conduct the reaction at 105°-120°C., whereby to achieve a rapid result without damage to the wool. The wool may be dry, or it may contain its natural moisture content, i.e., about 10-15%.

The time of reaction will depend on such factors as the solvent selected, the amount of zinc acetate, the temperature of reaction, and the degree of modifica-

tion desired. Thus the reaction may take anywhere from a few minutes to several hours. Usually, the reaction is continued for a time necessary to provide a weight increase (by the wool) of about 5-20%, preferably 10-15%.

After reaction of the wool with zinc acetate, the chemically-modified wool is preferably treated to remove unreacted zinc acetate. Thus the wool may be treated as by wringing, passage through squeeze rolls, centrifugation, etc., to remove the excess reagent. In place of such mechanical treatment, or in conjunction therewith, the modified wool may be extracted with an inert volatile solvent such as butanone, trichloroethylene, alcohol, and the like. Preferably, the extraction solvent is heated prior to use to facilitate removal of excess reactant. Successive extractions with different solvents may be used to ensure complete removal of all unreacted material. The treated wool is then dried in the usual manner.

Although the properties of the products of the invention indicate actual chemical combination of the wool with the zinc acetate (or at least the zinc moiety thereof) has taken place, it is not certain that this is the mechanism involved. It is believed that the zinc moiety reacts with the amino, imidazole, guanidino, hydroxyl, phenolic, and carboxyl groups of the wool, including cross-linking reactions. It may be, however, that other reactions occur and it is not intended to limit the invention to any theoretical basis.

It is to be noted that the reaction in accordance with the invention does not impair the wool fiber for its intended purpose, that is, for producing woven or knitted textiles, garments, etc. The process of the invention may be applied to wool in the form of fibers, as such, or in the form of threads, yarns, slivers, rovings, knitted or woven goods, felts, etc. The wool textiles may be white or dyed goods and may be of all-wool composition or blends of wool with other textile fibers such as cotton, regenerated cellulose, viscose, animal hair, etc.

**EXAMPLES**

The invention is further demonstrated by the following illustrative examples.

The wool used in the experiments set forth below was scoured, undyed wool, exhaustively extracted with trichloroethylene followed by ethanol, then dried for 70 minutes at 120°C. All weight increases are given on a dry wool basis. Zinc acetate was in the form of the dihydrate,  $Zn(C_2H_3O_2)_2 \cdot 2H_2O$ .

**EXAMPLE 1**

A circular sample (8.0 cm.) of dried wool fabric (1.2 g.), zinc acetate (0.20 g.), and DMF (6 ml.) were placed in a covered (but unsealed) Petri dish and held in an oven at 110°C. for 45 minutes. The treated wool sample was successively extracted with warm butanone and overnight with hot ethanol to remove unreacted material. The sample was then dried for 70 minutes at 120°C. and the weight increase was measured.

The reaction was repeated as above except that the amount of zinc acetate used was varied as follows: 0.80 g., 1.20 g., 1.60 g., and 3.20 g., respectively. The results of all the experiments are tabulated below.

| Zinc acetate, g. | Weight increase, % |
|------------------|--------------------|
| 0.20             | 5                  |
| 0.80             | 11                 |

-continued

| Zinc acetate, g. | Weight increase, % |
|------------------|--------------------|
| 1.20             | 11                 |
| 1.60             | 13                 |
| 3.20             | 16                 |

## EXAMPLE 2

A sample of dry wool fabric (1.2 g.), zinc acetate (1.5 g.), and DMF (6 ml.) were heated in a Petri dish at 110°C. at times tabulated below. The treated wool sample was extracted and dried as in Example 1.

The above procedure was repeated substituting either zinc chloride or zinc bromide.

The increase in dry weight of all samples is summarized below. The special value of zinc acetate is shown by the higher weight increase of the wool compared to zinc chloride and zinc bromide.

| Salt          | Weight increase, % |         |
|---------------|--------------------|---------|
|               | 45 min.            | 90 min. |
| Zinc acetate  | 13                 | 13      |
| Zinc chloride | 5                  | 5       |
| Zinc bromide  | 5                  | 6       |

## EXAMPLE 3

A sample of dry wool fabric (1.2 g.), zinc acetate (2.0 g.), and N-methyl-2-pyrrolidinone (6 ml.) were heated in a Petri dish at 110°C. for 45 minutes. The treated wool sample was extracted and dried as in Example 1.

The above procedure was repeated substituting either dimethyl sulfoxide or ethylene glycol in place of the N-methyl-2-pyrrolidinone.

The increase in dry weight of all samples was determined. The results are summarized below.

| Solvent                  | Weight increase, % |
|--------------------------|--------------------|
| N-Methyl-2-pyrrolidinone | 17                 |
| Dimethyl sulfoxide       | 12                 |
| Ethylene glycol          | 16                 |

## EXAMPLE 4

A swatch (24 × 14 cm.) of dried wool fabric (7.0 g.), zinc acetate (16.0 g.), and DMF (50 ml.) were placed in a 25 × 14 cm. pan. The pan was covered with a glass plate and held in an oven at 110°C. for 60 minutes. The treated wool sample was extracted and dried as in Example 1. The increase in dry weight of the wool was 15%. This product was tested as follows:

10 Insect resistance was tested on treated and untreated wool replicate fabric samples (0.5 g.) by exposing them to larvae of the black carpet beetle for 14 days. The average excrement weight from each sample was then measured. The results as tabulated below show the greatly increased insect resistance conferred by the treatment. The marked reduction of excrement with treated wool reflects the protection by the treatment against larval attack.

| Material tested          | Excrement per larva, mg. |
|--------------------------|--------------------------|
| Untreated wool (control) | 3.19                     |
| Product of the invention | 0.64                     |

Having thus described our invention, we claim:

1. A process for preparing modified wool which has increased resistance to insects, which comprises reacting wool with zinc acetate in the presence of N,N-dimethylformamide at a temperature of about from 105° to 120°C. until there is attained a weight increase by the wool of about from 5 to 20%.

2. A process for preparing modified wool which has increased resistance to insects, which comprises reacting wool with zinc acetate in the presence of N-methyl-2-pyrrolidinone at a temperature of about from 105° to 120°C. until there is attained a weight increase by the wool of about from 5 to 20%.

3. A process for preparing modified wool which has increased resistance to insects, which comprises reacting wool with zinc acetate in the presence of dimethyl sulfoxide at a temperature of about from 105° to 120°C. until there is attained a weight increase by the wool of about from 5 to 20%.

4. A process for preparing modified wool which has increased resistance to insects, which comprises reacting wool with zinc acetate in the presence of ethylene glycol at a temperature of about from 105° to 120°C. until there is attained a weight increase by the wool of about from 5 to 20%.

\* \* \* \* \*